

## [54] INSULATING DIELECTRIC FOR GAS DISCHARGE DEVICE

[75] Inventors: Roger E. Ernsthausen, Luckey; Michael E. Fein; Bernard W. Byrum, Jr., both of Toledo, all of Ohio

[73] Assignee: Owen-Illinois, Inc., Toledo, Ohio

[21] Appl. No.: 587,499

[22] Filed: Jun. 16, 1975

## Related U.S. Application Data

[60] Continuation-in-part of Ser. No. 291,956, Sep. 25, 1972, abandoned, which is a division of Ser. No. 217,395, Jan. 12, 1972, abandoned.

[51] Int. Cl.<sup>2</sup> ..... H01J 61/30; H01J 61/35

[52] U.S. Cl. ..... 313/220; 313/201;  
313/221

[58] Field of Search ..... 313/188, 220, 221, 201

## [56] References Cited

## U.S. PATENT DOCUMENTS

|           |         |                 |       |            |
|-----------|---------|-----------------|-------|------------|
| 3,334,269 | 8/1967  | L'Heureux       | ..... | 313/220 X  |
| 3,716,742 | 2/1973  | Nakayama et al. | ..... | 313/188 X  |
| 3,787,106 | 1/1974  | Schermerhorn    | ..... | 313/220 X  |
| 3,846,670 | 11/1974 | Schaufele       | ..... | 315/169 TV |
| 3,932,920 | 1/1976  | Ernsthausen     | ..... | 313/220 X  |

Primary Examiner—Palmer C. Demeo

Attorney, Agent, or Firm—Myron E. Click; David H. Wilson

## [57] ABSTRACT

There is disclosed a gas discharge device containing at least two electrodes, at least one of the electrodes being insulated from the gas by a dielectric member. There is particularly disclosed a multiple gaseous discharge display/memory panel having an electrical memory and capable of producing a visual display, the panel being characterized by an ionizable gaseous medium in a gas chamber formed by a pair of opposed dielectric material charge storage members, each of which is respectively backed by an array of electrodes, the electrodes behind each dielectric material member being oriented with respect to the electrodes behind the opposing dielectric material member so as to define a plurality of discrete discharge units.

At least one dielectric insulating member contains a predetermined beneficial amount of a source of at least one element selected from copper, silver, cadmium, mercury, and zinc.

The selected element or elements may be utilized in any suitable form, such as a compound, mineral, and/or elemental. Likewise, such may be incorporated into the dielectric by any suitable means, including being applied as a layer within the dielectric or on the surface thereof.

38 Claims, 6 Drawing Figures











## INSULATING DIELECTRIC FOR GAS DISCHARGE DEVICE

This is a continuation-in-part of copending U.S. Pat. Application Ser. No. 291,956 filed Sept. 25, 1972, now abandoned, which is a division of U.S. Patent Application Ser. No. 217,395 filed Jan. 12, 1972, now abandoned.

### BACKGROUND OF THE INVENTION

This invention relates to novel multiple gas discharge display/memory panels or units which have an electrical memory and which are capable of producing a visual display or representation of data such as numerals, letters, television display, radar displays, binary words, etc.

Multiple gas discharge display and/or memory panels of one particular type with which the present invention is concerned are characterized by an ionizable gaseous medium, usually a mixture of at least two gases at an appropriate gas pressure, in a thin gas chamber or space between a pair of opposed dielectric charge storage members which are backed by conductor (electrode) members, the conductor members backing each dielectric member typically being transversely oriented to define a plurality of discrete gas discharge units or cells.

In some prior art panels the discharge units are additionally defined by surrounding or confining physical structure such as by cells or apertures in perforated glass plates and the like so as to be physically isolated relative to other units. In either case, with or without the confining physical structure, charges (electrons, ions) produced upon ionization of the elemental gas volume of a selected discharge unit, when proper alternating operating potentials are applied to selected conductors thereof, are collected upon the surfaces of the dielectric at specifically defined locations and constitute an electrical field opposing the electrical field which created them so as to terminate the discharge for the remainder of the half cycle and aid in the initiation of a discharge on a succeeding opposite half cycle of applied voltage, such charges as are stored constituting an electrical memory.

Thus, the dielectric layers prevent the passage of substantial conductive current from the conductor members to the gaseous medium and also serve as collecting surfaces for ionized gaseous medium charges (electrons, ions) during the alternate half cycles of the A.C. operating potentials, such charges collecting first on one elemental or discrete dielectric surface area and then on an opposing elemental or discrete dielectric surface area on alternate half cycles to constitute an electrical memory.

An example of a panel structure containing non-physically isolated or open discharge units is disclosed in U.S. Pat. No. 3,499,167 issued to Theodore C. Baker, et al.

An example of a panel containing physically isolated units is disclosed in the article by D. L. Bitzer and H. G. Slottow entitled "The Plasma Display Panel — A Digitally Addressable Display With Inherent Memory," Proceeding of the Fall Join Computer Conference, IEEE, San Francisco, California, Nov. 1966, pages 541-547. Also reference is made to U.S. Pat. No. 3,559,190.

In the construction of the panel, a continuous volume of ionizable gas is confined between a pair of dielectric surfaces backed by conductor arrays forming matrix

elements. The cross conductor arrays may be orthogonally related (but any other configuration of conductor arrays may be used) to define a plurality of opposed pairs of charge storage areas on the surfaces of the dielectric bounding or confining the gas. Thus, for a conductor matrix having H rows and C columns the number of elemental discharge units will be the product H  $\times$  C and the number of elemental or discrete areas will be twice the number of such elemental discharge units.

In addition, the panel may comprise a so-called monolithic structure in which the conductor arrays are created on a single substrate and wherein two or more arrays are separated from each other and from the gaseous medium by at least one insulating member. In such a device the gas discharge takes place not between two opposing electrodes, but between two contiguous or adjacent electrodes on the same substrate; the gas being confined between the substrate and an outer retaining wall.

It is also feasible to have a gas discharge device wherein some of the conductive or electrode members are in direct contact with the gaseous medium and the remaining electrode members are appropriately insulated from such gas, i.e., at least one insulated electrode.

In addition to the matrix configuration, the conductor arrays may be shaped otherwise. Accordingly, while the preferred conductor arrangement is of the crossed grid type as discussed herein, it is likewise apparent that where a maximal variety of two dimensional display patterns is not necessary, as where specific standardized visual shapes (e.g., numerals, letters, words, etc.) are to be formed and image resolution is not critical, the conductors may be shaped accordingly, i.e., a segmented display.

The gas is one which produces visible light or invisible radiation which stimulates a phosphor (if visual display is an objective) and a copious supply of charges (ions and electrons) during discharge.

In prior art, a wide variety of gases and gas mixtures have been utilized as the gaseous medium in a gas discharge device. Typical of such gases include CO; CO<sub>2</sub>; halogens; nitrogen; NH<sub>3</sub>; oxygen; water vapor; hydrogen; hydrocarbons; P<sub>2</sub>O<sub>5</sub>; boron fluoride; acid fumes; TiCl<sub>4</sub>; Group VIII gases; air; H<sub>2</sub>O<sub>2</sub>; vapors of sodium, mercury, thallium, cadmium, rubidium, and cesium; carbon disulfide; laughing gas; H<sub>2</sub>S; deoxygenated air; phosphorus vapors; C<sub>2</sub>H<sub>2</sub>; CH<sub>4</sub>; naphthalene vapor; anthracene; freon; ethyl alcohol; methylene bromide; heavy hydrogen; electron attaching gases; sulfur hexafluoride; tritium; radioactive gases; and the rare or inert gases.

In one preferred practice hereof, the gas mixture comprises at least one rare gas, more preferably at least two rare gases, selected from neon, argon, xenon, and krypton. Beneficial amounts of mercury and/or helium may also be present.

In an open cell Baker, et al. type panel, the gas pressure and the electric field are sufficient to laterally confine charges generated on discharge within elemental or discrete dielectric areas within the perimeter of such areas, especially in a panel containing non-isolated units.

As described in the Baker, et al. patent, the space between the dielectric surfaces occupied by the gas is such as to permit photons generated on discharge in a selected discrete or elemental volume of gas to pass freely through the gas space and strike surface areas of dielectric remote from the selected discrete volumes,

such remote, photon struck dielectric surface areas thereby emitting electrons so as to condition at least one elemental volume other than the elemental volume in which the photons originated.

With respect to the memory function of a given discharge panel, the allowable distance or spacing between the dielectric surfaces depends, inter alia, on the frequency of the alternating current supply, the distance typically being greater for lower frequencies.

While the prior art does disclose gaseous discharge devices having externally positioned electrodes for initiating a gaseous discharge, sometimes called "electrodeless discharge," such prior art devices utilized frequencies and spacings or discharge volumes and operating pressures such that although discharges are initiated in the gaseous medium, such discharges are ineffective or not utilized for charge generation and storage at high frequencies; although charge storage may be realized at lower frequencies, such charge storage has not been utilized in a display/memory device in the manner of the Bitzer-Slottow or Baker, et al. invention.

The term "memory margin" is defined herein as

$$M. M. = (V_f - V_E)/(V_f/2)$$

where  $V_f$  is the half amplitude of the smallest sustaining voltage signal which results in a discharge every half cycle, but at which the cell is not bi-stable and  $V_E$  is the half amplitude of the minimum applied voltage sufficient to sustain discharges once initiated.

It will be understood that basic electrical phenomenon utilized in this invention is the generation of charges (ions and electrons) alternately storable at pairs of opposed or facing discrete points or areas on a pair of dielectric surfaces backed by conductors connected to a source of operating potential. Such stored charges result in an electrical field opposing the field produced by the applied potential that created them and hence operate to terminate ionization in the elemental gas volume between opposed or facing discrete points or areas of dielectric surface. The term "sustain a discharge" means producing a sequence of momentary discharges, one discharge for each half cycle of applied alternating sustaining voltage, once the elemental gas volume has been fired, to maintain alternate storing of charges at pairs of opposed discrete areas on the dielectric surfaces.

In accordance with the practice of this invention, there is incorporated into the dielectric of a gas discharge device a beneficial amount of a source of at least one element selected from copper, silver, cadmium, mercury, and zinc.

As used herein, the phrase "incorporated into" is intended to comprise any suitable means whereby a source of the selected element is appropriately combined with the dielectric, such as by intimately adding or mixing the source into the dielectric pre-melt batch or to the melt, by ion exchange; by ion implantation; by diffusion techniques; or by applying one or more layers to the charge storage surface of the dielectric, or to the electrode contact surface of the dielectric, or as an internal layer within the dielectric.

In one particular embodiment hereof, the source of the selected element is applied as one or more layers to the charge-storage surface of the dielectric.

As used herein, the term "layer" is intended to be all inclusive of other similar terms such as film, deposit, coating, finish, spread, covering, etc.

It is contemplated that the element source may be applied as a layer over one or more previously applied dielectric layers. Likewise, one or more layers of other substances may be applied over the layer of the element source. Such other dielectric layers may comprise luminescent phosphors and/or any other suitable compounds, especially inorganic compounds of Al, Pb, Si, Ti, Hf, rare earths (e.g., thorium), Group IA (e.g., cesium), and/or Group IIA (e.g., magnesium).

10 The source of the selected element is applied to the dielectric surface (or over a previously applied layer) by any convenient means including not by way of limitation vapor deposition; vacuum deposition; chemical vapor deposition, wet spraying upon the surface a mixture of a solution of the layer substance suspended or dissolved in a liquid followed by evaporation of the liquid; dry spraying of the layer upon the surface; thermal evaporation using direct heat, electron beam, or laser; plasma flame and/or arc spraying and/or deposition; and sputtering target techniques.

15 Each layer of the source of the selected element is applied to the dielectric, as a surface or sub-layer, in an amount sufficient to obtain the desired beneficial result, usually to a thickness of at least about 100 angstrom units, with a typical thickness range of about 200 angstrom units per layer up to about 1 micron (10,000 angstrom units) per layer.

20 In the fabrication of a gaseous discharge panel, the dielectric material is typically applied to and cured on the surface of a supporting glass substrate or base to which the electrode or conductor elements have been previously applied. The glass substrate may be of any suitable composition such as a soda lime glass composition. Two glass substrates containing electrodes and 25 cured dielectric are then appropriately sealed together, e.g., using thermal means, so as to form a panel.

25 In one preferred practice of this invention, each element containing layer is applied to the surface of the cured dielectric before the panel heat sealing cycle, with the substrate temperature during the layer application ranging from about 150° to about 600° F.

30 In accordance with the practice of this invention, it is contemplated using any suitable source of an element selected from copper, silver, cadmium, mercury, and zinc.

35 Typical sources include the elemental form of the selected element, a mineral, and/or a compound. It is especially contemplated using inorganic compounds.

40 Although insulating or semi-conductor materials are typically used, conductor materials may be used if the material is appropriately isolated within or on the dielectric so as not to be in electrical contact with a source of potential and/or ground.

45 Likewise if a conductive material is used in a multiple cell device, the geometric arrangement of the material may be such that no two cells are electrically connected by the conductive material. For example, a conductive material could be deposited as a spot over each discharge site.

50 The selected source is typically a solid. However, liquid materials may be used, especially if applied in a suitable binder.

55 Typical inorganic copper compounds include copper amine azide, copper diammine dichloride, copper hexammine dichloride, copper tetrammine dithionate, copper tetrammine nitrate, copper amine nitrate, copper tetrammine sulfate, tricopper antimonide, tricopper orthoarsenate, copper arsenide, tricopper arsenide, cop-

per orthoarsenite, copper azide, copper metaborate, copper boride, copper bromate, copper bromide, copper trioxybromide, copper carbonate, copper chlorate, copper perchlorate, copper chloride, copper chromate, copper dichromate, copper chromite, copper cyanide, copper ferricyanide, copper fluogallate, copper fluoride, copper fluosilicate, copper hydride, copper hydroxide, copper trihydroxychloride, copper trihydroxynitrate, copper iodate, copper paraperiodate, copper iodide, copper mercury iodide (alpha and beta), copper nitride, copper hyponitrite, copper oxide ( $CuO$ ,  $Cu_2O$ ), copper peroxide, copper suboxide, copper oxychloride, copper orthophosphate, tricopper phosphide, copper selenate, copper selenide ( $Cu_2Se$ ,  $CuSe$ ), copper selenite, copper silicide, copper sulfate, copper sulfide, copper sulfite, copper telluride, copper tellurite, copper thiocyanate, and copper tungstate.

Typical inorganic silver compounds include silver orthoarsenate, silver orthoarsenite, silver azide, silver tetraborate, silver bromate, silver bromide, silver carbonate, silver chlorate, silver perchlorate, silver chloride, silver chlorite, silver chromate, dichromate, dischromate, silver cyante, silver cyanide, silver ferricyanide, silver fluogallate, silver fluoride, silver disfluoride, disilver fluoride, silver fluosilicate, silver iodate, silver periodate, silver iodide, silver iodermercurate, silver trihydrogen paraperiodate, silver hyponitrite, silver permanganate, silver mercury iodide, silver nitrate, silver nitrite, silver nitroplatinite, silver nitroprusside, silver oxide, silver peroxide, silver metaphosphate, silver orthophosphate, silver pyrophosphate, silver perrhenate, silver selenate, silver selenide, silver sulfate, silver sulfide, silver sulfite, silver telluride, silver tellurite, silver thioantimonite, silver thioarsenite, silver thiocyanate, silver di-thionate, silver thiosulfate, silver tungstate and silver complexes such as diammine-silver perhenate.

Typical inorganic cadmium compounds include cadmium amide, cadmium ammonium chloride, cadmium ammonium sulfate, cadmium arsenide, cadmium borate, cadmium borotungstate, cadmium bromide, cadmium tetrabromide, cadmium carbonate, cadmium chlorate, cadmium chloride, cadmium tetrachloride, cadmium chloroplatinate, cadmium chromite, cadmium cyanide, cadmium ferrocyanide, cadmium fluogallate, cadmium fluoride, cadmium fluosilicate, cadmium hydroxide, cadmium iodate, cadmium iodide, cadmium permanganate, cadmium molybdate, cadmium nitrate, cadmium nitrocobaltate, cadmium oxalate, cadmium oxide, cadmium orthophosphate, cadmium pyrophosphate, cadmium phosphide, cadmium potassium cyanide, cadmium potassium sulfate, cadmium selenate, cadmium selenide, cadmium metasilicate, cadmium sulfate, cadmium sulfide, cadmium sulfite, cadmium telluride and cadmium tungstate.

Typical inorganic mercury compounds include mercury orthoarsenate, mercury azide, mercury bromate, mercury bromide, mercury bromide iodide, mercury carbonate, mercury chlorate, mercury chloride, mercury chromate, mercury cyanide, mercury fluoride, mercury fluosilicate, mercury iodate, mercury iodide, mercury nitrate, mercury nitrite, mercury nitride, mercury oxide, mercury oxybromide, mercury oxychloride, mercury oxycyanide, mercury oxyfluoride, mercury oxyiodide, mercury selenide, mercury sulfate, mercury sulfide, mercury orthotellurate, mercury thiocyanate, and mercury tungstate.

Typical inorganic zinc compounds include zinc aluminate, zinc amide, zinc antimonide, zinc orthoarsenate, zinc arsenite, zinc borate, zinc bromate, zinc bromide, zinc carbonate, zinc chlorate, zinc perchlorate, zinc chloride, zinc chloroplatinate, zinc chromate, zinc dichromate, zinc cyanide, zinc ferrate, zinc ferrocyanide, zinc fluoride, zinc fluosilicate, zinc gallate, zinc hydroxide, zinc iodate, zinc iodide, zinc permanganate, zinc nitrate, zinc nitride, zinc oxide, zinc peroxide, zinc orthophosphate, zinc pyrophosphide, zinc phosphide, zinc hypophosphite, zinc selenate, zinc selenide, zinc silicate, zinc metasilicate, zinc orthosilicate, zinc sulfate, zinc sulfide, zinc sulfite, zinc tellurate, zinc telluride, zinc thiocyanate, and zinc complexes such as diamminezinc chloride, tetrammine perrhenate, and tetrapyridine fluosilicate.

The use of this invention has many potential benefits. For example, sources of the selected element may be used alone or in combination with other elements (such as enumerated hereinbefore) to achieve lower panel operating voltages, thermal stability, more uniform panel operating voltages, decreased aging cycle time, etc.

Reference is made to the accompanying drawings and the figures thereon.

FIG. 1 is a partially cut-away plan view of a gaseous discharge display/memory panel as connected to a diagrammatically illustrated source of operating potentials,

FIG. 2 is a cross-sectional view (enlarged, but not to proportional scale since the thickness of the gas volume, dielectric members and conductor arrays have been enlarged for purposes of illustration) taken on lines 2 — 2 of FIG. 1,

FIG. 3 is an explanatory partial cross-sectional view similar to FIG. 2 (enlarged, but not to proportional scale),

FIG. 4 is an isometric view of a gaseous discharge display/memory panel,

FIG. 5 is a cross-sectional view similar to FIG. 3 illustrating a modification of the invention, and

FIG. 6 is a cross-sectional view similar to FIG. 3 illustrating a further modification of the invention.

The invention utilizes a pair of dielectric films 10 and 11 separated by a thin layer or volume of a gaseous discharge medium 12, the medium 12 producing a copious supply of charges (ions and electrons) which are alternately collectable on the surfaces of the dielectric members at opposed or facing elemental or discrete areas X and Y defined by the conductor matrix on non-gas-contacting sides of the dielectric members, each dielectric member presenting large open surface areas and a plurality of pairs of elemental X and Y areas. While the electrically operative structural members such as the dielectric members 10 and 11 and conductor matrixes 13 and 14 are all relatively thin (being exaggerated in thickness in the drawings) they are formed on and supported by rigid nonconductive support members 16 and 17 respectively.

Preferably, one or both of nonconductive support members 16 and 17 pass light produced by discharge in the elemental gas volumes. Preferably, they are transparent glass members and these members essentially define the overall thickness and strength of the panel. For example, the thickness of gas layer 12 as determined by spacer 15 is usually under 10 mils and preferably about 4 to 6 mils, dielectric layers 10 and 11 (over the conductors at the elemental or discrete X and Y areas) are usually between 1 and 2 mils thick, and conductors

13 and 14 about 8,000 angstroms thick. However, support members 16 and 17 are much thicker (particularly in larger panels) so as to provide as much ruggedness as may be desired to compensate for stresses in the panel. Support members 16 and 17 also serve as heat sinks for heat generated by discharges and thus minimize the effect of temperature on operation of the device. If it is desired that only the memory function be utilized, then none of the members need be transparent to light.

Except for being nonconductive or good insulators the electrical properties of support members 16 and 17 are not critical. The main function of support members 16 and 17 is to provide mechanical support and strength for the entire panel, particularly with respect to pressure differential acting on the panel and thermal shock. As noted earlier, they should have thermal expansion characteristics substantially matching the thermal expansion characteristics of dielectric layers 10 and 11. Ordinary 1/4 inch commercial grade soda lime plate glasses have been used for this purpose. Other glasses such as low expansion glasses or transparent devitrified glasses can be used provided they can withstand processing and have expansion characteristics substantially matching expansion characteristics of the dielectric coatings 10 and 11. For given pressure differentials and thickness of plates, the stress and deflection of plates may be determined by following standard stress and strain formulas (see R. J. Roark, *Formulas for Stress and Strain*, McGraw-Hill, 1954).

Spacer 15 may be made of the same glass material as dielectric films 10 and 11 and may be an integral rib formed on one of the dielectric members and fused to the other members to form a bakeable hermetic seal enclosing and confining the ionization gas volume 12. However, a separate final hermetic seal may be effected by a high strength devitrified glass sealant 15S. Tubulation 18 is provided for exhausting the space between dielectric members 10 and 11 and filling that space with the volume of ionizable gas. For large panels small beadlike solder glass spacers such as shown at 15B may be located between conductor intersections and fused to dielectric members 10 and 11 to aid in withstanding stress on the panel and maintain uniformity of thickness of gas volume 12.

Conductor arrays 13 and 14 may be formed on support members 16 and 17 by a number of well-known processes, such as photoetching, vacuum deposition, stencil screening, etc. In the panel shown in FIG. 4, the center-to-center spacing of conductors in the respective arrays is about 17 mils. Transparent or semi-transparent conductive material such as tin oxide, or aluminum can be used to form the conductor arrays and should have resistance less than 3000 ohms per line. Narrow opaque electrodes may alternately be used so that discharge light passes around the edges of the electrodes to the viewer. It is important to select a conductor material that is not attacked during processing by the dielectric material.

It will be appreciated that conductor arrays 13 and 14 may be wires or filaments of copper, silver or aluminum or any other conductive metal or material. For example 1 mil wire filaments are commercially available and may be used in the invention. However, formed in situ conductor arrays are preferred since they may be more easily and uniformly placed on and adhered to the support plates 16 and 17.

Dielectric layer members 10 and 11 are formed of an inorganic material and are preferably formed in situ as

an adherent film or coating which is not chemically or physically effected during bake-out of the panel. One such material is a solder glass such as Kimble SG-68 manufactured by and commercially available from the assignee of the present invention.

This glass has thermal expansion characteristics substantially matching the thermal expansion characteristics of certain soda-lime glasses, and can be used as the dielectric layer when the support members 16 and 17 are soda-lime glass plates. Dielectric layers 10 and 11 must be smooth and have a dielectric strength of about 1000 v. and be electrically homogeneous on a microscopic scale (e.g., no cracks, bubbles, crystals, dirt, surface films, etc.). In addition, the surfaces of dielectric layers 10 and 11 should be good photoemitters of electrons in a baked out condition. Alternatively, dielectric layers 10 and 11 may be overcoated with materials designed to produce good electron emission, as in U.S. Pat. No. 3,634,719, issued to Roger E. Ernsthausen. Of course, for an optical display at least one of dielectric layers 10 and 11 should pass light generated on discharge and be transparent or translucent and, preferably, both layers are optically transparent.

FIG. 5 illustrates one embodiment of the invention wherein a layer 410, 411 containing the source of at least one element selected from copper, silver, cadmium, mercury and zinc is applied over the dielectric layer 410a, 411a. A further embodiment is illustrated in FIG. 6 wherein a layer 510a, 511a is positioned between dielectric layers 510, 511 and 510b, 511b.

The preferred spacing between surfaces of the dielectric films is about 4 to 6 mils with conductor arrays 13 and 14 having center-to-center spacing of about 17 mils.

The ends of conductors 14-1 . . . 14-4 and support member 17 extend beyond the enclosed gas volume 12 and are exposed for the purpose of making electrical connection to interface and addressing circuitry 19. Likewise, the ends of conductors 13-1 . . . 13-4 on support member 16 extend beyond the enclosed gas volume 12 and are exposed for the purpose of making electrical connection to interface and addressing circuitry 19.

As in known display systems, the interface and addressing circuitry or system 19 may be relatively inexpensive line scan systems or the somewhat more expensive high speed random access systems. In either case, it is to be noted that a lower amplitude of operating potentials helps to reduce problems associated with the interface circuitry between the addressing system and the display/memory panel, per se. Thus, by providing a panel having greater uniformity in the discharge characteristics throughout the panel, tolerances and operating characteristics of the panel with which the interfacing circuitry cooperate, are made less rigid.

We claim:

1. In a gas discharge device containing at least two electrodes, at least one of the electrodes being insulated from the gas by a dielectric member, the improvement wherein at least one dielectric member contains an electrically non-conductive insulating source of at least one element selected from copper, silver, cadmium, mercury, and zinc.

2. The invention of claim 1 wherein the source of the element is contained within one or more layers on a surface of the dielectric member.

3. The invention of claim 1 wherein the source of the element is contained within one or more internal layers within the dielectric member.

4. The invention of claim 2 wherein the source of the element is contained within a dielectric layer having a thickness of at least 100 angstrom units.

5. The invention of claim 1 wherein the dielectric member is composed of a dielectric material and the source of the element is intimately mixed with the dielectric material.

6. The invention of claim 2 wherein the source of the element is contained within a dielectric layer having a thickness between about 200 and about 10,000 angstrom units.

7. The invention of claim 1 wherein said insulating source of at least one element selected from copper, silver, cadmium, mercury and zinc is an electrically non-conductive compound of said element.

8. The invention of claim 1 wherein said insulating source of copper is selected from the group of inorganic compounds consisting of copper amine azide, copper diammine dichloride, copper hexammine dichloride, copper tetrammine dithionate, copper tetrammine nitrate, copper amine nitrate, copper tetrammine sulfate, tricopper antimonide, tricopper orthoarsenate, copper arsenide, tricopper arsenide, copper orthoarsenite, copper azide, copper metaborate, copper boride, copper bromate, copper bromide, copper trioxybromide, copper carbonate, copper chlorate, copper perchlorate, copper chloride, copper chromate, copper dichromate, copper chromite, copper cyanide, copper ferricyanide, copper fluogallate, copper fluoride, copper fluosilicate, copper hydride, copper hydroxide, copper trihydroxychloride, copper trihydroxychloride, copper trihydroxy-nitrate, copper iodate, copper paraperiodate, copper iodide, copper mercury iodide, copper nitride, copper hyponitrite, copper oxide, copper peroxide, copper suboxide, copper oxychloride, copper orthophosphate, tricopper phosphide, copper selanate, copper selenide, copper selenite, copper silicide, copper sulfate, copper sulfide, copper sulfite, copper telluride, copper tellurite, copper thiocyanate, and copper tungstate.

9. The invention of claim 1 wherein said insulating source of silver is selected from the group of inorganic compounds consisting of silver orthoarsenate, silver orthoarsenite, silver azide, silver tetraborate, silver bromate, silver bromide, silver carbonate, silver chlorate, silver perchlorate, silver chloride, silver chlorite, silver chromate, silver dichromate, silver cyante, silver cyanide, silver ferricyanide, silver fluogallate, silver fluoride, silver fluosilicate, silver iodate, silver periodate, silver iodide, silver iodermercurate, silver trihydrogen paraperiodate, silver hyponitrite, silver permanganate, silver mercury iodide, silver nitrate, silver nitrite, silver nitroplatinite, silver nitroprusside, silver oxide, silver peroxide, silver metaphosphate, silver orthophosphate, silver pyrophosphate, silver perrhenate, silver selanate, silver selenide, silver sulfate, silver sulfide, silver sulfite, silver telluride, silver tellurite, silver thioantimonite, silver thioarsenite, silver thiocyanate, silver di-thionate, silver thiosulfate and silver tungstate and diammine-silver perrhenate.

10. The invention of claim 1 wherein said insulating source of cadmium is selected from the group of inorganic compounds consisting of cadmium amide, cadmium ammonium chloride, cadmium ammonium sulfate, cadmium arsenide, cadmium borate, cadmium borotungstate, cadmium bromide, cadmium tetraboramide, cadmium carbonate, cadmium chlorate, cadmium chloride, cadmium tetrachloride, cadmium chloroplatinate, cadmium chromite, cadmium cyanide, cad-

mium ferrocyanide, cadmium fluogallate, cadmium fluoride, cadmium fluosilicate, cadmium hydroxide, cadmium rodate, cadmium iodide, cadmium permanganate, cadmium molybdate, cadmium nitrate, cadmium nitrocobaltate, cadmium oxalate, cadmium oxide, cadmium orthophosphate, cadmium pyrophosphate, cadmium phosphide, cadmium potassium cyanide, cadmium potassium sulfate, cadmium selenate, cadmium selenide, cadmium metasilicate, cadmium sulfate, cadmium sulfide, cadmium sulfite, cadmium telluride and cadmium tungstate.

11. The invention of claim 1 wherein said insulating source of mercury is selected from the group of inorganic compounds consisting of mercury orthoarsenate, mercury azide, mercury bromate, mercury bromide, mercury bromide iodide, mercury carbonate, mercury chlorate, mercury chloride, mercury chromate, mercury cyanide, mercury fluoride, mercury fluosilicate, mercury iodate, mercury iodide, mercury nitrate, mercury nitrite, mercury nitride, mercury oxide, mercury oxybromide, mercury oxychloride, mercury oxycyanide, mercury oxyfluoride, mercury oxyiodide, mercury selenide, mercury sulfate, mercury sulfide, mercury orthotellurate, mercury thiocyanate, and mercury tungstate.

12. The invention of claim 1 wherein insulating source of zinc is selected from the group of inorganic compounds consisting of zinc aluminate, zinc amide, zinc antimonide, zinc orthoarsenate, zinc arsenite, zinc borate, zinc bromate, zinc bromide, zinc carbonate, zinc chlorate, zinc perchlorate, zinc chloride, zinc chloroplatinate, zinc chromate, zinc dichromate, zinc cyanide, zinc ferrate, zinc ferrocyanide, zinc fluoride, zinc fluosilicate, zinc gallate, zinc hydroxide, zinc iodate, zinc iodide, zinc permanganate, zinc nitrate, zinc nitride, zinc oxide, zinc peroxide, zinc orthophosphate, zinc pyrophosphate, zinc phosphide, zinc hypophosphate, zinc selenate, zinc selenide, zinc silicate, zinc metasilicate, zinc orthosilicate, zinc sulfate, zinc sulfide, zinc sulfite, zinc tellurate, zinc telluride, zinc thiocyanate and zinc complexes such as diamminezinc chloride, tetrammine perrhenate, and tetrapyridine fluosilicate.

13. In a multiple gaseous discharge display/memory panel having an electrical memory and capable of producing a visual display, the panel being characterized by an ionizable gaseous medium in a gas chamber formed by a pair of opposed dielectric material charge storage members, each of which dielectric members is respectively backed by an array of electrodes, the electrodes behind each dielectric member being oriented with respect to the electrodes behind the opposing dielectric member so as to define a plurality of discrete discharge units, the improvement wherein at least one dielectric member contains an electrically non-conductive insulating source of at least one element selected from copper, silver, cadmium, mercury, and zinc.

14. The invention of claim 13 wherein the source is contained within one or more layers on a surface of the dielectric member.

15. The invention of claim 13 wherein the source is contained with one or more internal layers within the dielectric member.

16. The invention of claim 13 wherein the source is in the form of an inorganic oxide.

17. The invention of claim 14 wherein the source of the element is contained within a dielectric layer having a thickness of at least 100 angstrom units.

18. The invention of claim 14 wherein the source of the element is contained within a dielectric layer having a thickness of about 200 to about 10,000 angstrom units.

19. The invention of claim 13 wherein the dielectric member is composed of a dielectric material and the source of the element is intimately mixed with the dielectric material.

20. The invention of claim 13 wherein said insulating source of at least one element selected from copper, silver, cadmium, mercury and zinc is an electrically non-conductive compound of said element.

21. The invention of claim 13 wherein said insulating source of copper is selected from the group of inorganic compounds consisting of copper amine azide, copper diammine dichloride copper hexammine dichloride, copper tetrammine dithionate, copper tetrammine nitrate, copper amine nitrate, copper tetrammine sulfate, tricopper antimonide, tricopper orthoarsenate, copper arsenide, tricopper arsenide, copper orthoarsenite, copper azide, copper metaborate, copper boride, copper bromate, copper bromide, copper trioxybromide, copper carbonate, copper chlorate, copper perchlorate, copper chloride, copper chromate, copper dichromate, copper chromite, copper cyanide, copper ferricyanide, copper fluogallate, copper fluoride, copper fluosilicate, copper hydride, copper hydroxide, copper trihydroxychloride, copper trihydroxychloride, copper trihydroxynitrate, copper iodate, copper paraperiodate, copper iodide, copper mercury iodide, copper nitride, copper hyponitrite, copper oxide, copper peroxide, copper suboxide, copper oxychloride, copper orthophosphate, tricopper phosphide, copper selanate, copper selenide, copper selenite, copper silicide, copper sulfate, copper sulfide, copper sulfite, copper telluride, copper tellurite, copper thiocyanate, and copper tungstate.

22. The invention of claim 13 wherein said insulating source of silver is selected from the group of inorganic compounds consisting of silver orthoarsenate, silver orthoarsenite, silver azide, silver tetraborate, silver bromate, silver bromide, silver carbonate, silver chlorate, silver perchlorate, silver chlorate, silver chlorite, silver chromate, silver dichromate, silver cyante, silver cyanide, silver ferricyanide, silver fluogallate, silver fluoride, silver difluoride, disilver fluoride, silver fluosilicate, silver iodate, silver periodate, silver iodide, silver iodermercurate, silver trihydrogen paraperiodate, silver hyponitrite, silver permanganate, silver mercury iodide, silver nitrate, silver nitrite, silver nitroplatinate, silver nitroprusside, silver oxide, silver peroxide, silver metaphosphate, silver orthophosphate, silver pyrophosphate, silver perrhenate, silver selanate, silver selenide, silver sulfate, silver sulfide, silver sulfite, silver telluride, silver tellurite, silver thioantimonite, silver thioarsenite, silver thocyanate, silver di-thionate, silver thiosulfate, silver tungstate and diammine-silver perrhenate.

23. The invention of claim 13 wherein said insulating source of cadmium is selected from the group of inorganic compounds consisting of cadmium amide, cadmium ammonium chloride, cadmium ammonium sulfate, cadmium arsenide, cadmium borate, cadmium borotungstate, cadmium bromide, cadmium tetrabromide, cadmium carbonate, cadmium chlorate, cadmium chloride, cadmium tetrachloride, cadmium chloroplatinate, cadmium chromite, cadmium cyanide, cadmium ferrocyanide, cadmium fluogallate, cadmium fluoride, cadmium fluosilicate, cadmium hydroxide, cadmium rodite, cadmium iodide, cadmium permanganate, cadmium molybdate, cadmium nitrate, cadmium nitroco-

baltate, cadmium oxalate, cadmium oxide, cadmium orthophosphate, cadmium pyrophosphate, cadmium phosphide, cadmium potassium cyanide, cadmium potassium sulfate, cadmium selenate, cadmium selenide, cadmium metasilicate, cadmium sulfate, cadmium sulfide, cadmium sulfite, cadmium telluride and cadmium tungstate.

24. The invention of claim 13 wherein said insulating source of mercury is selected from the group of inorganic compounds consisting of mercury orthoarsenate, mercury azide, mercury bromate, mercury bromide, mercury bromide iodide, mercury carbonate, mercury chlorate, mercury chloride, mercury chromate, mercury cyanide, mercury fluoride, mercury fluosilicate, mercury iodate, mercury iodide, mercury nitrate, mercury nitrite, mercury nitride, mercury oxide, mercury oxybromide, mercury oxychloride, mercury oxycyanide, mercury oxyfluoride, mercury oxyiodide, mercury selenide, mercury sulfate, mercury sulfide, mercury orthotellurate, mercury thiocyanate, and mercury tungstate.

25. The invention of claim 13 wherein insulating source of zinc is selected from the group of inorganic compounds consisting of zinc aluminate, zinc amide, zinc antimonide, zinc orthoarsenate, zinc arsenite, zinc borate, zinc bromate, zinc bromide, zinc carbonate, zinc chlorate, zinc perchlorate, zinc chloride, zinc chloroplatinate, zinc chromate, zinc dichromate, zinc cyanide, zinc ferrate, zinc ferrocyanide, zinc fluoride, zinc fluosilicate, zinc gallate, zinc hydroxide, zinc iodate, zinc iodide, zinc permanganate, zinc nitrate, zinc nitride, zinc oxide, zinc peroxide, zinc orthophosphate, zinc pyrophosphide, zinc phosphide, zinc hypophosphite, zinc selenate, zinc selenide, zinc silicate, zinc metasilicate, zinc orthosilicate, zinc sulfate, zinc sulfide, zinc sulfite, zinc tellurate, zinc telluride, zinc thiocyanate and zinc complexes such as diammin zinc chloride, tetrammine perrhenate, and tetrapyridine fluosilicate.

26. In the operation of a gaseous discharge display/memory device characterized by an ionizable gaseous medium in a gas chamber formed by a pair of opposed dielectric material charge storage members, each of which dielectric members is respectively backed by an array of electrodes, the electrodes behind each dielectric member being oriented with respect to the electrodes behind the opposing dielectric member so as to define a plurality of discrete discharge units, the improvement which comprises substantially decreasing the operating voltages and aging cycle time and providing thermal stability and more uniform panel operating voltages by incorporating into at least one of said dielectric members an electrically non-conductive, insulating source of at least one element selected from copper, silver, cadmium, mercury and zinc.

27. The invention of claim 26 wherein the dielectric member comprises a dielectric material and the source of the element is intimately mixed with the dielectric material.

28. The invention of claim 26 wherein the source of the element is contained within at least one layer on a surface of the dielectric member.

29. The invention of claim 26 wherein the source of the element is contained within at least one internal layer within the dielectric member.

30. The invention of claim 28 wherein the source of the element is contained within a dielectric layer having a thickness of at least 100 angstrom units.

31. The invention of claim 28 wherein the source of the element is contained within a dielectric layer having a thickness of about 200 to about 10,000 angstrom units.

32. The invention of claim 26 wherein the dielectric member is composed of a dielectric material and the source of the element is intimately mixed with the dielectric material.

33. The invention of claim 26 wherein said insulating source of at least one element selected from copper, silver, cadmium, mercury and zinc is an electrically non-conductive compound of said element.

34. The invention of claim 26 wherein said insulating source of copper is selected from the group of inorganic compounds consisting of copper amine azide, copper diammine dichloride, copper hexammine dichloride, copper tetrammine dithionate, copper tetrammine nitrate, copper amine nitrate, copper tetrammine sulfate, tricopper antimonide, tricopper orthoarsenate, copper arsenide, tricopper arsenide, copper orthoarsenide, copper azide, copper metaborate, copper boride, copper bromate, copper bromide, copper trioxybromide, copper carbonate, copper chlorate, copper perchlorate, copper chloride, copper chromate, copper dichromate, copper chromite, copper cyanide, copper ferricyanide, copper fluogallate, copper fluoride, copper fluosilicate, copper hydride, copper hydroxide, copper trihydroxychloride, copper trihydroxychloride, copper trihydroxynitrate, copper iodate, copper paraperiodate, copper iodide, copper mercury iodide, copper nitride, copper hyponitrite, copper oxide, copper peroxide, copper suboxide, copper oxychloride, copper orthophosphate, tricopper phosphide, copper selenate, copper selenide, copper selenite, copper silicide, copper sulfate, copper sulfide, copper sulfite, copper telluride, copper tellurite, copper thiocyanate, and copper tungstate.

35. The invention of claim 26 wherein said insulating source of silver is selected from the group of inorganic compounds consisting of silver orthoarsenate, silver orthoarsenite, silver azide, silver tetraborate, silver bromate, silver bromide, silver carbonate, silver chlorate, silver perchlorate, silver chloride, silver chlorite, silver chromate, silver dichromate, silver cyanate, silver cyanide, silver ferricyanide, silver fluogallate, silver fluoride, silver difluoride, disilver fluoride, silver fluosilicate, silver iodate, silver periodate, silver iodide, silver iodermercurate, silver trihydrogen paraperiodate, silver hyponitrite, silver permanganate, silver mercury iodide, silver nitrate, silver nitrite, silver nitroplatinite, silver nitroprusside, silver oxide, silver peroxide, silver metaphosphate, silver orthophosphate, silver pyrophosphate, silver perrhenate, silver selenate, silver selenide, silver sulfate, silver sulfide, silver sulfite, silver telluride, silver tellurite, silver thioantimonite, silver thioarsenite,

nite, silver thiocyanate, silver di-thionate, silver thiosulfate, silver tungstate and diammine-silver perrhenate.

36. The invention of claim 26 wherein said insulating source of cadmium is selected from the group of inorganic compounds consisting of cadmium amide, cadmium ammonium chloride, cadmium ammonium sulfate, cadmium arsenide, cadmium borate, cadmium borotungstate, cadmium bromide, cadmium tetrabromide, cadmium carbonate, cadmium chlorate, cadmium chloride, cadmium tetrachloride, cadmium chloroplatinate, cadmium chromite, cadmium cyanide, cadmium ferrocyanide, cadmium fluogallate, cadmium fluoride, cadmium fluosilicate, cadmium hydroxide, cadmium rodate, cadmium iodide, cadmium permanganate, cadmium molybdate, cadmium nitrate, cadmium nitrocobaltate, cadmium oxalate, cadmium oxide, cadmium orthophosphate, cadmium pyrophosphate, cadmium phosphide, cadmium potassium cyanide, cadmium potassium sulfate, cadmium selenate, cadmium selenide, cadmium metasilicate, cadmium sulfate, cadmium sulfide, cadmium sulfite, cadmium telluride and cadmium tungstate.

37. The invention of claim 26 wherein said insulating source of mercury is selected from the group of inorganic compounds consisting of mercury orthoarsenate, mercury azide, mercury bromate, mercury bromide, mercury bromide iodide, mercury carbonate, mercury chlorate, mercury chloride, mercury chromate, mercury cyanide, mercury fluoride, mercury fluosilicate, mercury iodate, mercury iodide, mercury nitrate, mercury nitrite, mercury nitride, mercury oxide, mercury oxybromide, mercury oxychloride, mercury oxycyanide, mercury oxyfluoride, mercury oxyiodide, mercury selenide, mercury sulfate, mercury sulfide, mercury orthotellurate, mercury thiocyanate, and mercury tungstate.

38. The invention of claim 26 wherein insulating source of zinc is selected from the group of inorganic compounds consisting of zinc aluminate, zinc amide, zinc antimonide, zinc orthoarsenate, zinc arsenite, zinc borate, zinc bromate, zinc bromide, zinc carbonate, zinc chlorate, zinc perchlorate, zinc chloride, zinc chloroplatinate, zinc chromate, zinc dichromate, zinc cyanide, zinc ferrate, zinc ferrocyanide, zinc fluoride, zinc fluosilicate, zinc gallate, zinc hydroxide, zinc iodate, zinc iodide, zinc permanganate, zinc nitrate, zinc nitride, zinc oxide, zinc peroxide, zinc orthophosphate, zinc pyrophosphate, zinc phosphide, zinc hypophosphite, zinc selenate, zinc selenide, zinc silicate, zinc metasilicate, zinc orthosilicate, zinc sulfate, zinc sulfide, zinc sulfite, zinc tellurate, zinc telluride, zinc thiocyanate and zinc complexes such as diamminezinc chloride, tetrammine perrhenate, and tetrapyridine fluosilicate.

\* \* \* \* \*